

## UNITED STATES PATENT OFFICE

2,014,238

WHITE CAST IRON ALLOY AND METHOD  
OF MAKING THE SAME

Frank A. Raven, Albany, and Clarence D. Foulke,  
Buffalo, N. Y., assignors to Industrial Furnace  
Corporation, Buffalo, N. Y., a corporation of  
New York

No Drawing. Application January 15, 1932,  
Serial No. 586,952

## 2 Claims. (Cl. 148—21.7)

This invention relates to alloys of white cast iron, and it has particular reference to a white iron alloy, containing, in addition to the usual ingredients, alloying elements in such proportions as to render the iron readily amenable to heat treatment to yield an article having desirable physical properties.

Heretofore it has been the general practice to make white iron castings with carbon and silicon, and manganese and sulphur, in such proportions as to yield, upon heat treatment, the material known as malleable cast iron. Such material, as a commercial article, has been made with a tensile strength of something less, on the average, of 55,000 pounds per square inch, with elongations of the order of twelve to twenty per cent in two inches. Metallurgically, malleable cast iron is composed of free iron or ferrite, interspersed with temper carbon. Aside from the constituents named above, phosphorus is also usually present, but other impurities have been avoided in general foundry practice.

The factors considered in the making of malleable cast iron have been, that the carbon must be originally present as combined carbon, or cementite, that the silicon must not be too high, lest the criterion of combined carbon be defeated, albeit the silicon should be present in appreciable amounts to facilitate the subsequent breakdown of the cementite, or, in other words, to accelerate the annealing or graphitizing action. These matters have led to certain limits and ratios for carbon and silicon; thus, if the carbon be 2.45 per cent, the silicon may be about 0.84 per cent, and if the carbon be 2.10 per cent, the silicon should be about 1.06 per cent.

Likewise, the manganese and sulphur, both of which are known as retardants of the annealing process, should not be too high, lest the heat treatment be necessarily extended. Foundry practice, however, imposes limits on the sulphur, and the manganese value has been made somewhat more than twice the sulphur, it having been found that while these two elements, separately, exert a retarding effect, in proper proportions conjointly they neutralize each other. In practice, sulphur values of about 0.06 to 0.10 per cent have been tolerated, with the manganese running to about 0.3 per cent; the exact figures varying, of course, with foundry conditions and the type of casting desired.

It has more recently been discovered that, if the white iron casting is modified in its composition to contain an available excess of retardant, as, for example, an excess of manganese, to

about say 0.6 to 1.5 per cent, and such castings are subjected to certain heat treating operations, it is possible to obtain a commercial metal, differing materially from malleable cast iron in its metallurgical aspect, as well as chemical composition, and also having greatly enhanced physical properties. In the practice of this process, it has been observed that the time of heat treatment of the white iron casting, necessary to effect the breakdown of the free cementite, 5 may run for an appreciable time, say about twenty-four hours at 1700° F. This length of time may be objectionable for economic or commercial reasons. It has also been observed, moreover, that the castings made by the process referred to are open to the general objection of low corrosion resistance as compared to "malleable" cast iron or other metals and alloys, and this factor militates against the use of the articles in certain applications where the strength is 10 desired.

We have discovered that heat treated white iron castings of enhanced physical properties, comparable to those obtained in the castings containing excess retardant, may be obtained, however, in shorter periods of time, and with increased resistance to corrosion, by alloying in the white iron casting a combination of elements, which facilitate the breakdown of free cementite, and so lessen the time of heat treatment required, but which combination does not, however, effect a like influence on the decomposition of combined cementite or pearlite. In this connection, it may be explained that the conversion of hard and non-ductile white iron into 15 a more ductile and strong material is thought to be due to the decomposition of the combined carbon or cementite. This cementite occurs in two conditions, first, as free or massive cementite, which is decomposed above certain temperature 20 ranges, generally called the "critical". The balance of the cementite occurs in the form of pearlite, which is broken down by heat at temperatures below the critical. Our invention is predicated upon the principle of modifying the 25 normal white iron composition by the inclusion of elements which do not retard or prevent the actions occurring above the critical, but which do exert such effect on the actions below the critical, so that physical changes may take place 30 in preference to the chemical change which has been sought heretofore in making malleable cast iron. The invention further involves the principle of utilizing, as the modifying means, elements which impart to the casting, in its final 35

form, enhanced physical properties and a greater resistance to corrosion.

More specifically, we have discovered that if the composition of the iron be modified by the 5 addition of chromium and copper, the desired results may be obtained. In this connection, it may be noted that, heretofore, chromium has been recognized as a retardant for the annealing actions, and the effect of chromium, when 10 present to any appreciable extent, is so marked that its presence is shunned by the white iron manufacturer or founder. Copper, on the other hand, has been stated by some to be a retardant 15 of the annealing operation, and by others an accelerator, and published reports of the addition of copper have indicated that it is not efficacious in increasing the strength of the heat treated casting. Whatever may be the truth or 20 merits of these several views, we are able to utilize these elements to advantage, for we have discovered that, at temperatures of treatment above the critical, the accelerating effect of copper predominates, so that a shorter time of heat treatment 25 may be employed, whereas, at temperatures below the critical, the accelerating effect of copper is so minimized as not to interfere with the 30 preferential progress of the physical actions, desired in imparting to the casting the enhanced physical properties. We have further found that this combination of elements imparts to the final casting an increased resistance to corrosive action.

In speaking just above of copper, it will, of course, be understood that reference is made to 35 the effect of the copper present with other elements, such as the retardants chromium or manganese. If copper alone is employed, it appears that the accelerating influence prevails at temperatures both above and below the critical, while 40 if chromium alone is used, the retarding effect is such as to render difficult any annealing at all. The two specifics, conjointly, however, well attain the object of accelerating the high temperature 45 reaction, without interfering with the low temperature changes desired to obtain the final product herein contemplated.

As exemplary of the results to be obtained, the following data, derived from the testing of sample bars of white cast iron, may be noted.

| Chemical composition | Alloy No. 1 | Alloy No. 2 | Alloy No. 3    |
|----------------------|-------------|-------------|----------------|
| Carbon.....          | 2.00        | 2.00        | 2.00           |
| Silicon.....         | 1.06        | 1.06        | 1.06           |
| Manganese.....       | 0.85        | 0.85        | 0.85           |
| Sulphur.....         | 0.072       | 0.072       | 0.072          |
| Chromium.....        | 0.07        | 0.07        | 0.07           |
| Copper.....          | 0.00        | 0.00        | 2.00 (approx.) |

80 Samples of each alloy were subjected to a heat treatment at 1700° F. for periods of time of 10, 15, and 26 hours, the last time being that which would be used (approximately) in the high temperature heat treatment of this alloy, if neither chromium or copper were present, but if the manganese value were high, as in the instant cases. Microscopic examination of Alloy No. 1 showed that the free cementite was not broken down in any of the three heats, thereby showing that, taken alone, or with the manganese, a pronounced retarding effect was obtained with the addition of chromium. Alloy No. 2, however, showed nearly complete breakdown of the massive cementite, after heat treatment for only ten 85 hours, thereby showing that the addition of cop-

per had produced a resultant accelerating effect at the high temperature hold, while in Alloy No. 3, complete breakdown obtained in ten hours. After twenty-six hours' treatment, Alloy No. 3 showed a "bull's-eye" structure, indicating that 90 an excess of copper over that required for best results, in view of the chromium content, had been included.

Alloys No. 1 and No. 2 were then subjected to a low temperature heat treatment at 1300° F. for 10, twenty hours, or that which, with manganese present but chromium and copper absent, could be expected to give a material having a spheroidized structure with an ultimate strength in the neighborhood of 90,000 pounds. The values 15 obtained were, for Alloy No. 1, ultimate strength 86,100, yield point, 66,300, elongation 3.5 per cent. These figures indicate that the retarding effect of chromium was still pronounced, since the physical properties are not as much as they should 20 be, if no chromium were present. With Alloy No. 2, the following values were obtained, ultimate, 91,800, yield point 69,600, elongation, nine per cent, or about what could be anticipated if neither 25 chromium or copper were present. These results indicate that the deleterious retarding effect of the chromium, taken alone, had been eliminated, and, also, that the undue accelerating effect of the copper (if taken alone) had been arrested at the low temperature hold. It is also to be noted 30 that the effect noted by some for copper, namely, negligible improvement in strength, does not occur here. These elements, copper and chromium, moreover, impart increased corrosion resistance to the finished castings, thereby rendering such 35 materials available for wide range of service.

From the foregoing explanation, it will now be apparent that our invention provides for the heat treatment of white iron castings of modified composition in shorter periods of time than those 40 heretofore deemed permissible for commercial practice, by so modifying the alloy as to include elements which do not retard the breakdown of free cementite, but which permit of preferential progress of physical actions at temperatures at 45 which combined cementite tends to decompose. These alloys, as it will be noted, are of high strength and appreciable ductility, and are also highly resistant to corrosive influences. Those skilled in the art will understand, of course, that 50 the percentages of the various ingredients of the casting may be modified from the values hereinabove given, and it is not intended, therefore, to limit the invention to the specific compositions or heat treatments set forth. It is intended that 55 the invention should be considered in the light of the following claims.

We claim:

1. The method of making an iron alloy from white cast iron which comprises forming a white 60 cast iron containing carbon in the form of cementite, silicon, manganese, sulphur and phosphorus as normal constituents, and also an excess of manganese with chromium and copper, the 65 respective proportions of excess manganese, chromium and copper being such as to exert a retarding effect on the decomposition of combined cementite at heat treating temperatures below the critical, but exerting substantially no retarding effect on the breakdown of massive cementite 70 at heat treating temperatures above the critical, subjecting the iron to a temperature above the critical but below the temperature of incipient fusion for a length of time sufficient to decompose the massive cementite and to develop tem- 75

per carbon, cooling the casting, and subjecting the casting to heat treatment below the critical and at a temperature at which further changes in the casting occur, the manganese content being 5 between 0.6 and 1.5 per cent, the chromium content being of the order of one-tenth the copper, and the copper being not more than 2 per cent.

2. A heat treated and ductile white iron containing silicon, manganese, and sulphur in the proportions normally occurring in malleable white iron with an excess of manganese to make 10

the total manganese content between 0.6 and 1.5 per cent, said iron also containing temper carbon derived from cementite but being substantially free from graphitic carbon and massive cementite, said iron further containing limited amounts of chromium and copper, the amount of copper being not more than two per cent and the amount of chromium being of the order of one tenth the amount of copper. 5

FRANK A. RAVEN.  
CLARENCE D. FOULKE. 10